

# UNITED STATES PATENT OFFICE.

JAMES R. ROSE, OF EDGEWORTH, PENNSYLVANIA, AND JOHN HARRIS, OF LAKEWOOD, OHIO, ASSIGNEES TO CARBO-OXYGEN COMPANY, OF PITTSBURGH, PENNSYLVANIA, A CORPORATION OF DELAWARE.

## GASEOUS FUEL.

1,404,222.

Specification of Letters Patent. Patented Jan. 24, 1922.

No Drawing.

Application filed December 26, 1919. Serial No. 347,449.

To all whom it may concern:

Be it known that we, (1) JAMES R. ROSE, (2) JOHN HARRIS, citizens of the United States, residing at (1) Edgeworth, (2) Lakewood, in the county of (1) Allegheny, (2) Cuyahoga, and State of (1) Pennsylvania, (2) Ohio, have invented a certain new and useful Improvement in Gaseous Fuel, of which the following is a full, clear, and exact description.

This invention relates to gaseous fuel, and more particularly to a fuel which is especially adapted for the purpose of cutting metals with great rapidity, where extreme cleanliness of cutting is not essential. A use for which our gas is particularly well suited is for the cutting of scrap iron.

We obtain a gas having the above desirable characteristics by mixing with hydrogen as a combustible base, by-product coke-oven gas and butane in the proportions of from  $2\frac{1}{2}\%$  to  $12\frac{1}{2}\%$  by volume each of such by-product coke-oven gas and such propane to the hydrogen constituent. The by-product coke-oven gas has nearly the same flame temperature as the hydrogen, and the mixture of the butane therewith makes the temperature of the combined gases in excess of that obtained by the combustion of hydrogen alone and equal to at least  $3200^{\circ}$  C. Furthermore, the by-product coke-oven gas is also readily obtainable as a source of gas for cutting purposes in steel mills. The gaseous mixture produces within the burning hydrogen a visible cone which enables the operator to adjust the proportions of the gases and of the combustion-supporting oxygen as may be necessary, as well as to apply the flame in the most advantageous manner to the work.

Both the volume of the flame and the heat units produced by the combustion of the mixture are greater than are produced by the combustion of hydrogen alone, but are lower than usually required for operating on heavy masses of metal and for cutting cast iron and steel and corroded, dirty and slaggy iron and steel. However, our gaseous mixture is capable of cutting with much greater rapidity than can be accomplished by gases having such higher carbon content.

Taking Koppers's by-product coke-oven

gas as a type, the average analysis of the same is as follows:

|                                                                     |      |
|---------------------------------------------------------------------|------|
| CO <sub>2</sub> -----                                               | 2.6  |
| Illuminants -----                                                   | 4.3  |
| Oxygen -----                                                        | 0.2  |
| CO -----                                                            | 6.3  |
| Hydrogen -----                                                      | 46.3 |
| CH <sub>4</sub> -----                                               | 35.0 |
| Nitrogen -----                                                      | 5.3  |
| B. T. U. -----                                                      | 630  |
| Cu. ft. of oxygen required for combustion of a cu. ft. of gas ----- | 1.09 |

According to Richards on Metallurgical Calculations, published in 1908, and with the by-product coke-oven gas of approximately the analysis above set forth, the flame temperature produced by the combustion of the above described gaseous mixture will be about  $3200^{\circ}$  C., and the variations in the percentages of the said gases will cause approximately the following variations in the net B. T. U. per cu. ft. of mixture and in the cubic feet of oxygen required for the combustion of a cubic foot of such mixture:

No. 1 mixture, 95% H. with  $2\frac{1}{2}\%$  each of by-product coke-oven gas and butane; net B. T. U.'s 373; cu. ft. of oxygen .662.

No. 2 mixture, 75% H. with  $12\frac{1}{2}\%$  each of by-products coke-oven gas and butane; net B. T. U.'s 692; cu. ft. of oxygen 1,312.

Having thus described our invention, what we claim is:—

1. A gas for cutting, welding and heating purposes consisting of a mixture of by-product coke gas and butane with hydrogen in the proportions of from  $2\frac{1}{2}\%$  to  $12\frac{1}{2}\%$  by volume of each of by-product coke gas and butane to hydrogen.

2. A gas for cutting, welding and heating purposes consisting of a mixture of by-product coke-oven gas and butane with hydrogen in proportions not substantially less than 5% by volume of such combined gases to the hydrogen and not materially more than 25% of such combined gases to the hydrogen, the by-product coke-oven gas and butane being present in the proportions of at least  $2\frac{1}{2}\%$  each in such mixture.

In testimony whereof we hereunto affix our signatures.

JAMES R. ROSE.  
JOHN HARRIS.